

# UNITED STATES PATENT OFFICE.

LEIGH S. BACHE, OF BOUND BROOK, NEW JERSEY.

## PROCESS OF TREATING AND COLORING WOOD AND PRODUCT OF SUCH PROCESS.

1,077,252.

Specification of Letters Patent.

Patented Nov. 4, 1913.

No Drawing.

Application filed July 6, 1911. Serial No. 637,207.

To all whom it may concern:

Be it known that I, LEIGH S. BACHE, a citizen of the United States, and a resident of Boundbrook, in the county of Somerset and State of New Jersey, have invented a Process of Treating and Coloring Wood and Product of Such Process, of which the following is a specification.

The invention relates to the treatment of wood or like fiber which may be used in the arts for various purposes without liability of change due to atmospheric or other conditions and the sustaining of a permanent homogeneous color throughout the wood or fiber.

The object of the invention is to produce a colored wood impervious to moisture and colored through and through.

A further object is to provide a vehicle for thoroughly impregnating wood or fiber and simultaneously using therewith a color which will hold and bind the impregnating material.

It is not new in the art to stain wood and fiber nor is it new in the art to impregnate to a greater or lesser extent such material with a water-proofing compound or a fire-proofing compound. So far as known to applicant, such impregnation and coloring has acted only to certain depths upon the material. For instance, in impregnation and coloring of wood the surface and what might be called a skin of varying thickness receives the treatment, but if cross-sawed or cut there is non-uniformity in the coloring conditions as well as in the impregnation. It follows that the articles to be treated must be treated in given sizes and the impregnation will be substantially uniform up to certain depths from the surface on all parts of the article.

It is one of the principal objects of the present invention to thoroughly and completely impregnate the wood or fiber through and through and at the same time color it to any desired degree for any use to which it may be desired to utilize it.

In carrying out the process, wood or similar fibrous material is used as the base which is to be treated and must be in a substantially dry condition to secure the quickest and best results in treatment. Wood which is suitably seasoned or kiln-dried may be readily treated and will, after subjection to the process hereinafter defined, maintain a constant condition both as to color and

holding qualities with reference to the impregnating materials.

In carrying out the process, various materials may be used, including a combination of waxes of different characters, of mineral, vegetable or animal origin combined with the products derived from volatile oils or produced by oxidization of hydro-carbons such as rosins and mixed with stearic acid or its ethers or glycerins or the commercial form of stearin, so-called stearic acid. The above materials are used in conjunction with suitable coloring materials preferably those which are soluble in oils, such as one having an indulin base made soluble with stearin or olein. Very excellent results have been obtained by mixing a quantity of carnauba wax with paraffin, resin and coloring matter. The ingredients vary somewhat with the treatment to be produced but in any event the waxes, paraffin and rosins act as a conveyer for thoroughly impregnating the material with the coloring matter and when combined as hereinafter set forth act as a binder with the coloring matter so that the article treated has a definite and constant value of impregnating materials and coloring matter.

In treating wood and fiber various artistic results may be secured by utilizing different coloring materials producing the various tints such as oak, mahogany, ebony, birch, maple, walnut, and in fact almost any of the natural woods and when the wood is once treated it may be readily polished and finished without staining other than that introduced at the time of treatment. Furthermore, the treatment has this great advantage, namely, that it shows any imperfections in the material to be treated. For instance, where wood is of imperfect form and has a streak of "tight-grain" or "dry-rot" or "sap-grain," the color will immediately disclose the fact that the wood has not been properly impregnated and light streakings will show. Thus it is possible to ascertain before attempting to use the finished product that it is a perfect piece of wood suitable for fine work, fine veneer cutting, etc.

In carrying out the process, the following ingredients are used: Saturated hydro-carbon of the general series having the formula  $C_nH_{2n}+2$  in solid form, such as paraffin having a melting point between 40° and 60° C. and boiling at 120° C. or higher; an animal, mineral or vegetable wax preferably

carnauba wax; an oxidized hydro-carbon having a low melting point such as rosin; stearic acid; coloring materials preferably such as are soluble in oil and in the menstruum employed for saturation. These ingredients are mixed in varying proportions, excellent results having been attained by a mixture as follows: paraffin 100 lbs., carnauba wax 20 lbs., rosin 20 lbs., coloring matter,  $3\frac{1}{2}$  lbs., in some cases using a comparatively small proportion by weight of stearic acid. They are reduced by subjecting to heat in a suitable vessel until raised to the boiling point. Thereupon, the material to be treated is boiled in the mixture until it attains a gravity sufficient to carry it to the bottom of the caldron. This is the best indication that the material is thoroughly impregnated.

It has been found that wood treated in this manner shows no appreciable change of condition under varying atmospheric conditions, will not absorb moisture, and will not evaporate its impregnating solution. Apparently the coloring and impregnating material bind one another in the fiber of the wood and the impregnating material carries the color completely through the fiber so that it may be cut in any form, always showing uniform color and complete impregnation.

Obviously, the proportion of ingredients might be varied and substitutions might be made without departing from the spirit or intent of the invention.

What I claim as my invention and desire to secure by Letters Patent is:

1. The herein described process of treating wood and fiber which consists in boiling said wood or fiber in a solution of saturated hydro-carbon, wax, oxidized hydro-carbon, stearic acid and coloring matter, said boiling being continued until the gravity of

the wood or fiber is greater than that of the solution.

2. The herein described process of treating wood and fiber which consists in subjecting said wood or fiber to a boiling bath of paraffin, carnauba wax, rosin and coloring matter soluble in the said menstruum with substantially equal parts by weight of carnauba wax and rosin and an excess of paraffin.

3. A new product consisting of a solid fibrous body impregnated through and through with saturated hydrocarbon, wax, oxidized hydrocarbon and a coloring matter that is soluble in the menstruum composed of said ingredients, the said saturating ingredients co-acting to cause a uniform saturation and also to prevent flow of the impregnating materials within the said body after it has been saturated.

4. A new product consisting of a solid fibrous body impregnated through and through with saturated hydrocarbon, wax, oxidized hydrocarbon, stearic acid, and a coloring matter that is soluble in the menstruum composed of said ingredients, the said saturating ingredients co-acting to cause a uniform saturation and also to prevent flow of the impregnating materials within the said body after it has been saturated.

5. A new product consisting of a solid fibrous body impregnated through and through with a compound of saturated hydrocarbon, wax, oxidized hydrocarbon and a coloring matter soluble in the menstruum composed of said ingredients, the specific gravity of the product being greater than that of the impregnating medium.

LEIGH S. BACHE.

Witnesses:

A. LANG,  
GEO. T. SMALLEY.